

3,304,191

## COAL TAR PAVING COMPOSITIONS AND PROCESS FOR PREPARING THEM

Richard C. Barrett, New Milford, N.J., assignor to Allied Chemical Corporation, New York, N.Y., a corporation of New York  
No Drawing. Filed May 21, 1963, Ser. No. 282,143  
5 Claims. (Cl. 106—279)

This invention relates to improved coal tar compositions adapted for use as paving binders, and to a process for preparing them.

Bituminous materials have been used for many years in the preparation of road paving compositions to bind mineral aggregate in the roadbed or other paved areas and to present a smooth and durable wearing surface for traffic.

Bituminous binders of two main type are used in paving operations. The most widely used are the asphalts, derived as residues from asphaltic petroleums. The petroleum asphalts are normally solid, or semi-solid bitumens, which are usually applied to the road or other similar surface or to mineral aggregate either in the hot molten state or as solutions in volatile solvents. Such compositions then "set" or solidify, either rapidly, by cooling or, more slowly, by evaporation of the volatile solvent, thus producing firm surfaces which are little affected by temperature changes which occur in normal outdoor exposure, resulting in surfaces possessing low "temperature susceptibilities." The petroleum asphalts, in general, however, suffer both from poor initial wetting power for the mineral aggregate used in pavement construction which results in poor binding of the aggregate mass. They also suffer from poor water resistance, so that when exposed to water they tend to disengage from the aggregate. The asphaltic bitumens, moreover, are completely soluble in petroleum oils and greases and, thus, surfaces composed of such binders suffer serious damage when exposed to such petroleum products, as for example, to jet fuel, gasoline or motor oil and the like.

Also used as bituminous paving binders are certain tarry residues obtained in the distillation of crude tars resulting from the destructive distillation of bituminous coal, the principal source of such tar being the by-product coke ovens producing metallurgical coke. Such residues may be, and usually are, cut back or fluxed, before use, with coal tar distillates to meet the required specifications for the desired type of tar. Standard road tars are customarily prepared in fourteen different grades, which are essentially similar except for differences in consistency or viscosity, the variety of grades being provided so that material may be chosen to meet local conditions of temperature, road conditions, climate, etc. Specifications for such tars are given in ASTM specification D-490. The lower numbered grades RT-1, RT-2, RT-3 and RT-4, are relatively low viscosity tars used in general in prime coat application and light surface treatment of pavements; RT-5 and RT-6 are of somewhat higher consistency and serve for use in surface treatment and road mix; RT-7, RT-8 and RT-9 of still higher consistencies, are useful in surface treatment, road mix, plant mix and seal coats, these latter grades being the most widely used and representative grades of road tars; RT-10, RT-11 and RT-12 of even higher consistencies are for use in surface treatment, plant mix, penetration, crack filler and seal coat applications, while the special grades RT CB-5 and RT CB-6 of consistencies similar to the RT-5 and RT-6 grades but somewhat quicker setting, are used in patching, surface treatment and also for plant mix and road mix where low temperature application and quick setting are desired.

All these coal tar derived road tars have superior wetting power for mineral aggregate and are extremely resistant to both water and to petroleum oils and greases. The coal tars, however, lack the low temperature susceptibility of the petroleum asphaltic bitumens, and tend to flow and bleed out of the aggregate when used in paving construction.

The asphalt type binders used in road and similar constructions are essentially non-volatile and are ordinarily applied as hot melts or as solvent solutions. When hot applied, these materials set by cooling and undergo no further change in physical characteristics. When applied as a solution in a solvent the binder cures by solvent evaporation and leaves a residual film of the non-volatile asphalt.

10 The coal tar binders, in contrast, are composed of a multiplicity of components with varying degrees of volatility. Although often heated to increase fluidity for application, they are not initially solid at normal temperature, and harden or cure by the slow progressive evaporation of the more volatile portions of the tar itself. When attempts are made to hasten the curing time by increasing the amount of the more volatile component there must also be an increase in the hard non-volatile component 15 if the desired viscosity is to be retained. The non-volatile pitch constituents of coal tar have a high temperature susceptibility and thus such a blend, while having a satisfactory cure rate will leave a residual binder highly susceptible to changes in consistency with changes in temperature.

20 An object of the present invention is to provide a paving composition composed entirely of coal tar derived components, which has an unusually low temperature susceptibility and an exceptionally fast rate of curing when applied to road or other surfaces.

25 These and other objects are accomplished by the new compositions of my invention comprising mixtures of normal road tars with between about 25% and about 75% by volume of an oxidized aromatic flux oil residue, as 30 hereinafter defined, fluxed with sufficient quantities of a coal tar distillate fluxing oil to meet the requirements of ASTM specifications D-490.

35 The coal tar paving compositions of my invention are suitable for use in all types of paving applications, for 40 example, in the preparation of bituminous macadam, bituminous concrete, in cover coats and in the preparation of the so-called "black bases." The advantages of these black bases have recently been demonstrated by road tests conducted by the American Association of State Highway 45 Officials. "Black bases" are pre-mixed blends of run-of-bank gravel of the desired size, with bituminous paving compositions. Such bases are applied alone or in combination with penetration macadam to the sub-base of the area to be paved.

50 Use of these black bases has been found to yield economic advantages in that they require lower coat thicknesses to provide the same load bearing capacity, than are required of the standard penetration macadam or bituminous concrete. The greater the load bearing capacity of 55 the black base, the thinner the layer that can be applied to produce the same durability in the paving. These black bases, moreover, are customarily stock piled at the job site in advance of starting construction so that for 60 such black bases, it is important that the tar used in their preparation be selected to preserve the workability of the base over the period of storage.

65 Besides meeting all the requirements of the ASTM standards, the paving compositions of my invention all have unusually low "temperature susceptibilities," fast 70 curing rates, and yield residues of controlled high softening points.

"Temperature susceptibility," as used in the bituminous

paving art, refers to the change in consistency of the composition with temperature. Thus a composition which is hard at low temperatures may soften rapidly as temperature is raised. Such a composition is said to have a high temperature susceptibility. A composition with a low temperature susceptibility, on the other hand, will not soften as rapidly with rises in temperature and will not harden as rapidly with reductions in temperature. This susceptibility to changes in consistency with temperature may be rated by the correlation of the needle penetration at a given temperature, usually at 77° F., to the ring and ball softening point of the bitumen. A common and useful method of correlating these values is by the so-called "Penetration Index," as defined in the publication entitled, "Classifying Asphalts by Means of Penetration Index," by J. Ph. Pfeiffer and P. M. Van Doormal which appeared in the February 23, 1938 issue of "National Petroleum News," pages R-78 to R-84.

In that publication a nomograph is provided relating penetration to ring and ball softening temperature, from which a "penetration index" value may be derived which is a valuable index of temperature susceptibility of the bitumen. The temperature susceptibility scale as shown in the publication ranges from minus 10 to plus 20. An index of +20 would indicate zero temperature susceptibility. With increasing susceptibility the index decreases through 0 to -10, the latter value corresponding to an infinitely large susceptibility. Thus the lower the penetration index, the higher is the temperature susceptibility of the bitumen.

Penetration indexes of normal coal tar based road tars meets the ASTM specifications usually range substantially below -1.5 usually close to -2, and hence are rated as having high temperature susceptibility, i.e., poor resistance to temperature change. By the incorporation of substantial proportions of oxidized aromatic flux oil as defined, in normal road tar, the penetration index is significantly raised to values above -2.0, usually to values between about -1.5 and about -1.0 or higher.

The term "curing rate" refers to the rate of gradual hardening or setting of the tar, after application to the surface, which takes place by evaporation of volatile matter in the tar. This rate depends on a number of factors, including the relative proportions of components of different boiling points, ambient temperatures during the successive stages of cure, etc. A rapid cure to the consistency required to minimize bleeding or flow and to sustain traffic is desirable.

As a measure of curing rate, ASTM specification D-490 requires that the residue produced by distilling the road tar to 300° C. according to ASTM test method D-20 shall have a ring and ball softening point between 30° C. and 70° C., the tars of higher residue softening point values being the faster curing. The precise range varies slightly for the different grades of tar. As a practical matter the majority of road tars have residue softening points of around 40 to 45, and thus have relatively low curing rates. While it is possible to produce a "normal" road tar having high residue softening points up to the 70° C. maximum or higher by the simple expedient of removing some of the lower boiling components of the tar by distillation to a high melting point residue and then diluting or "cutting back" the tar with a volatile solvent, the resulting residues as deposited on the road or other surface have excessively high temperature susceptibilities and are subject to embrittlement on cooling to normal ambient temperatures and below.

The tars of the present invention, on the other hand, have residue softening points in the upper portion of the ASTM-D-490 specification range, i.e. between about 50° C. and about 70° C. and still provide residues having a low degree of temperature susceptibility as pointed out above. Thus the tars of my invention possess concomitantly the two heretofore-considered paradoxical properties of fast cure and low temperature susceptibilities rendering

them of exceptional value particularly in a number of specialized applications as brought out above.

While the ring and ball softening point of the D-20 distillation residue, obtained as outlined above, is indicative of the relative curing rates to be expected of normal tars as presently formulated, the test fails to simulate actual curing conditions by so great a measure that it might be possible to prepare a tar which would meet the above tests but which still would not cure properly, when deposited on the road or other surface. To meet this deficiency and to provide a definitive test which more accurately reflects the actual behavior of the tar when exposed to atmospheric conditions on the road, or other surface, an accelerated test has recently been devised to measure curing rates which can be expected of tars under normal conditions on a road or other surface. This test involves applying a uniform, thin film of the tar of standard thickness, usually 0.032 inch, to a plane surface, and subjecting the films to simulated aging conditions by exposure to 50° C. (122° F.) temperature under forced air circulation conditions, and measuring the ring and ball softening points of the films at successive intervals. In this way a definitive and substantially reliable comparison of relative curing times of different tars can be obtained.

25 The oxidized aromatic flux oil residue which is the critical component of the new paving tars of my invention, is obtained by subjecting a selected coal tar flux oil to intimate contact with a gas containing elemental oxygen, for example air, at temperatures between about 200° C. and about 500° C. for a time sufficient to produce an oxidized flux oil residue containing at least about 15%, preferably between about 15% and about 45% by weight of benzol-insoluble compounds, usually about 30%. The oxidized aromatic flux oil residue is a pitch-like material

30 having a ring and ball softening point between about 50° C. and about 135° C., preferably between about 60° C. and about 90° C. and a Penetration Index between 0 and -1.5, usually about -0.5. The oxidized product has a specific gravity, Sp. Gr. 25/25° C., between

35 1.20 and 1.25, usually about 1.22. As noted above, the flux oil after oxidation, no longer is an oil but has substantially the characteristics of a pitch. Blowing the flux oil under the above conditions gives rise to formation of benzol-insoluble compounds which are believed to be responsible for the improved characteristics of reduced temperature susceptibilities in the residues from the blended tars containing the oxidized aromatic flux oil residue. Quinoline-insolubles, on the other hand, are not formed in this treatment, and so are present in the treated residue

40 in proportions of not more than about 5%.

The selected flux oils from which the oxidized product is derived, are distillate oils obtained in the distillation of tars resulting from the destructive distillation of bituminous coals. These oils boil above about 250° C. under standard conditions, and usually comprise the so-called light and heavy tar oil fractions, and may also include residues from redistillation of lighter distillate fractions.

Proportions of the oxidized aromatic flux oil residue as defined, up to 75% by volume based on the volume of the normal road tar/air-blown flux oil blend may be used. I have found that higher proportions of oxidized aromatic flux oil residue tend to cause crystallization of the resulting film when applied to the surface and, in the higher consistency grades (RT-7 to RT-12), prevent compliance with the ASTM float test requirement due to this crystallization tendency. Even small proportions of the oxidized aromatic flux oil residue added to normal road tars improve the temperature susceptibility and cure of the resulting blend. However, I usually prefer to use at least about 25% of oxidized aromatic flux oil residue with 75% tar, percentages between about 50% and about 75% based on the oxidized aromatic flux oil residue/normal tar blend being preferred.

The blends of oxidized aromatic flux oil residue with normal tar are then cut back with a suitable fluxing agent

## 5

to the consistency desired. Suitable fluxing agents are those in the nature of the so-called light carbolic oil residue (LCOR) which is a coal tar fraction boiling primarily (85% dry) between about 235° C. and about 315° C., suitably having a specific gravity, Sp. Gr. 25/25° C., between about 1.040 and about 1.060, usually obtained, as the name implies, as a residue from distillation of the light carbolic oil fraction of the coal tar. Other coal tar derived fluxing agents may also be used having the same general character as the light carbolic oil residue, for example, a similar oil which may be obtained as the distillate produced by stripping creosote oil to a vapor temperature of 300° C., or if desired, a mixture of creosote oil and light carbolic oil residue meeting the above boiling range specification may be used.

In general, a suitable fluxing agent is a coal tar distillate of which at least about 90% boils between about 210° C. and about 355° C. and having no more than about 10% residue above 355° C.

The resulting blends are useful in all paving applications for which the standard road tars are used, and provide resultant coatings which cure more rapidly than standard coatings, have improved (reduced) temperature susceptibilities when cured, and result in higher melting coatings of characteristically high water resistance and good binding power for mineral aggregates.

The compositions of my invention preferably have distillation residues which have penetration indices as defined, of above -2, preferably between about -1.0 and about -0.5 and softening points of at least about 45° C., preferably between about 50° C. and about 70° C. These compositions also preferably have curing rates such that they achieve a softening point of at least about 40° C. in not more than about 5 days when exposed in a film 0.032 inch in thickness to forced air circulation at 50° C.

The following specific examples further illustrate my invention.

*Examples 1 and 2*

Two road tars were prepared by blending oxidized aromatic flux oil residue in the proportion of 25% and 50% with 75% and 50%, respectively, of standard road tar RT-8, and fluxing the resultant blends with light carbolic oil residues to RT-8 consistencies. The resulting blends had the properties shown in Table I below as compared to ASTM D-490 standards and the properties of the standard RT-8 used.

TABLE I

|                                                                    | ASTM Spec. D-490 | RT-8  | Ex. 1 | Ex. 2 |
|--------------------------------------------------------------------|------------------|-------|-------|-------|
| Percent RT-8                                                       |                  | 100   | 67    | 40.5  |
| Percent Oxidized Aromatic Flux Oil Residue                         |                  |       | 22.4  | 40.5  |
| Percent Light-Carbolic-Oil Residue                                 |                  |       | 10.6  | 19    |
| Specific Gravity at 25/25° C., min.                                | 1.14             | 1.200 | 1.19  | 1.18  |
| Float Test at 32° C., sec.                                         | 80-120           | 96.5  | 85    | 95    |
| Soluble in CS <sub>2</sub> , Percent, min.                         | 78               | 91.9  | 88.4  | 84.9  |
| Distillation Test (ASTM D-20), Percent Distillate by Weight, max.: |                  |       |       |       |
| 0-170° C.                                                          | 1.0              | 6.6   | 9.1   | 11.6  |
| 0-270° C.                                                          | 15.0             | 6.6   | 9.1   | 11.6  |
| 0-300° C.                                                          | 25.0             | 15.9  | 21.6  | 25.2  |
| Residue, Percent                                                   |                  | 83.2  | 77.9  | 74.1  |
| Softening Point of Residue (Ring and Ball), °C                     | 35-70            | 43.2  | 49.1  | 57.3  |

The road tars prepared as described above were then distilled according to ASTM method D-20 to such end point temperature as to produce residues melting within the range of 57°-58° C. (ring and ball). The residues from these distillations were then tested for softening point

## 6

(ring and ball) and penetration with the following results, shown in Table II below.

TABLE II

|                                                 | RT-8  | Ex. 1 | Ex. 2 |
|-------------------------------------------------|-------|-------|-------|
| Percent RT-8                                    | 100   | 67    | 40.5  |
| Percent Oxidized Aromatic Flux Oil Residue      |       | 22.4  | 40.5  |
| Percent Light Carbolic-Oil Residue              |       | 10.6  | 19    |
| Distillation:                                   |       |       |       |
| 0-300° C.                                       |       |       | 25.2  |
| 0-312° C.                                       | 24.2  | 25.8  |       |
| 0-330° C.                                       | 75.5  | 73.5  | 74.1  |
| Residue, Weight Percent                         |       |       |       |
| Softening Point of Residue (Ring and Ball), °C. | 57.0  | 58.0  | 57.3  |
| Penetration at 77° F./100 g./5 sec.             | 14    | 16    | 24    |
| Penetration Index                               | -1.99 | -1.60 | -1.06 |

These data show that the temperature-susceptibilities of the equi-melting residues are decreased as the amount of oxidized aromatic flux oil residue is increased.

The standard road binder and that of Example 2 were applied to aluminum panels in 0.032" thickness and heated in an oven at 50° C. The softening points of the residual films were determined at intervals with results shown in Table III below.

TABLE III

|                                                | RT-8 | Ex. 2 |
|------------------------------------------------|------|-------|
| Percent RT-8                                   | 100  | 40.5  |
| Percent Oxidized Aromatic Flux Oil Residue     |      | 40.5  |
| Percent Light-Carbolic-Oil Residue             |      | 19.0  |
| Softening Point after Heating Time (days) °C.: |      |       |
| 1.                                             | 26.6 | 36.0  |
| 2.                                             | 31.4 | 46.6  |
| 3.                                             | 35.4 | 52.6  |
| 4.                                             | 37.0 | 54.0  |
| 7.                                             | 42.4 | 55.0  |
| 10.                                            | 45.0 | 62.4  |

The above data show that the blended composition of Example 2, containing oxidized aromatic flux oil residue, although of the same softening point as the Standard RT-8 binder at the time of application, will set or cure more rapidly, as indicated by the more rapid attainment of high softening points, than will the standard road tar.

The oxidized aromatic flux oil residue used in the road tars of Examples 1 and 2 above was prepared by air blowing at 295°-300° C. and at air rate of 0.03 c.f.m./45 gallon of charge, a selected flux oil having the following properties:

ASTM-D-246 distillation percent dist. to:

|         |     |
|---------|-----|
| 210° C. | 0.0 |
| 235° C. | 0.0 |
| 270° C. | 3.4 |

315° C. ----- 32.7  
 355° C. ----- 81.6  
 Residue ----- 18.0  
 Specific gravity 25/25° C. ----- 1.101  
 Benzene insolubles ----- 0.5%

The oxidized aromatic flux oil residue used in Examples 1 and 2 had the following properties:

|                                 |      |       |
|---------------------------------|------|-------|
| Softening point (ring and ball) | C.   | 73.6° |
| Penetration at:                 |      |       |
| 77° F., 100 g., 5 sec.          |      | 8     |
| 77° F., 200 g., 30 sec.         |      | 25    |
| 115° F., 50 g., 5 sec.          |      | 37    |
| Penetration index               |      | -0.2  |
| Viscosity SSF at 300° F.        | sec. | 220   |
| Benzene insolubles              |      | 28.9  |
| Specific gravity                |      | 1.230 |

The light carbolic oil residue used in the above examples had the following properties:

|                               |         |       |
|-------------------------------|---------|-------|
| Specific gravity at 25/25° C. |         | 1.056 |
| D-246 distillation (° C.):    | Percent |       |
| 0-210                         |         | 0.0   |
| 0-235                         |         | 0.3   |
| 0-270                         |         | 64.3  |
| 0-315                         |         | 86.6  |
| 0-355                         |         | 93.3  |
| Residue                       |         | 5.5   |

### Example 3

An aromatic flux oil having the characteristics set out above was blown with air in a continuous manner at temperatures ranging from 300° C.-400° C. and pressures of 50-66 p.s.i.g. The resultant residue product was mixed continuously with a predetermined blend of normal road tar RT-10 and light carbolic oil residue of the character employed in the foregoing examples until the consistency fell within the range of ASTM test D-490 for RT-10. The normal tar used and the blend obtained were tested for compliance with ASTM requirements and for Penetration Index values as shown below.

|                                              | ASTM   | Standard | Ex. 3<br>Blend |
|----------------------------------------------|--------|----------|----------------|
| Regular RT-10, Volume Percent                |        | 100      | 34.7           |
| Air Blown Residue, Volume Percent            |        |          | 47.1           |
| Light Carbolic Oil Residue, Volume Percent   |        |          | 18.2           |
| Specific Gravity at 25° C., min.             | 1.15   | 1.232    | 1.213          |
| Float at 50° C.                              | 75-100 | 93       | 97             |
| Soluble CS <sub>2</sub> , min.               | 75     | 87.2     | 79.5           |
| ASTM Distillation (D-20), max.:              |        |          |                |
| 0-170° C.                                    | 1.0    | 0.0      | 0.0            |
| 0-270° C.                                    | 10     | 3.6      | 4.9            |
| 0-300° C.                                    | 20     | 9.1      | 17.4           |
| Softening Point Residue (Ring and Ball) ° C. | 40-70  | 40.2     | 49.2           |
| Penetration Residue 77° C./100 g./5 sec.     |        | 67       | 40             |
| Penetration Index                            |        | -3.7     | -1.9           |

To characterize the residue used in preparing this blended road tar, small samples of the air-blown residue stream were taken at frequent intervals and combined to form a composite sample representative of the air-

blown residue used in the blend. The composite sample was tested and found to have the following properties:

|                                   |  |       |
|-----------------------------------|--|-------|
| Sp. Gr. 25°/25° C.                |  | 1.237 |
| Soft. Pt. ring and ball, ° F.     |  | 166   |
| Distillation (° C.):              |  |       |
| First drop                        |  | 305   |
| 0-300, percent                    |  | 0     |
| 0-355, percent                    |  | 43.7  |
| 0-360, percent                    |  | 47.9  |
| Penetration, 77° F./100 g./5 sec. |  | 4     |
| Penetration index                 |  | -1.0  |
| Benzene insolubles percent        |  | 26.2  |

The standard RT-10 road tar and the oxidized aromatic flux oil residue-containing blend characterized above were applied to a test road on a fall day in Michigan. The standard and experimental road tars were applied from a standard tar spreader at a temperature of 225° F. and at a rate of 1/4 gallon per square yard. Immediately after application to the road, the tar was covered with 31B cover stone conforming to the specification

|                    |         |
|--------------------|---------|
|                    | Percent |
| Passing—3/8" sieve | 100     |
| No. 4 sieve        | 35-65   |
| No. 10 sieve       | 0-15    |

The cover stone was applied at the rate of 30 pounds per square yard and was immediately rolled with a ten ton roller.

Examination of the two test strips the following May on a day when the ambient temperature was in the low 80's showed that the standard RT-10 strip was bleeding badly whereas the strip containing oxidized aromatic flux oil residue binder was satisfactory. Sand was applied to the bleeding RT-10 strip in an amount to furnish 10 pounds of sand per square yard in an attempt to soak up the fluid binder, but was unsuccessful in relieving the condition, and the strip remained very slippery.

The two test strips were examined again, in September, two years after application. The regular RT-10 was found to exhibit some bleeding even after three coverings with sand. The blend containing oxidized aromatic flux oil residue binder had had no sand coverings and showed no evidence of bleeding. Both strips showed good adherence and no signs of failing except for a few cracks.

### Examples 4-7

Four road tars were prepared by blending mixtures of the same air-blown aromatic flux oil residue as used in Examples 1 and 2 and a standard RT-9 road tar containing between 40% and 60% air-blown residue with different fluxing oils, including (1) creosote oil, (2) creosote oil distillate to 300° C. and (3) light carbolic oil residue. These tars had the compositions shown in Table IV below.

TABLE IV

|                                                | ASTM<br>D 490 | RT-9  | Ex. 4 | Ex. 5 | Ex. 6 | Ex. 7 |
|------------------------------------------------|---------------|-------|-------|-------|-------|-------|
| RT-9                                           |               | 100   | 25.7  | 25.0  | 24.4  | 50.0  |
| Air-Blown Residue                              |               |       | 51.3  | 51.3  | 53.6  | 35.5  |
| Creosote Oil                                   |               |       | 23.0  |       | 5.4   |       |
| LCO R                                          |               |       |       |       | 16.6  | 14.5  |
| Creosote Distillate to 300° C.                 |               |       |       | 23.6  |       |       |
| Float Test at 32° C., sec.                     | 120-200       | 135   | 163   | 123   | 170   | 120   |
| CS <sub>2</sub> Soluble, Percent, min.         | 78            | 87.7  | 82.4  | 82.4  | 81.6  | 84.0  |
| Specific Gravity at 25/25° C., min.            | 1.14          | 1.218 | 1.203 | 1.162 | 1.191 | 1.202 |
| ASTM D-20 Dist.:                               |               |       |       |       |       |       |
| 0-270° C., wt. percent, max.                   | 15            | 6.2   | 2.3   | 9.3   | 11.1  | 11.2  |
| 0-300° C., wt. percent, max.                   | 25            | 15.8  | 10.9  | 22.3  | 22.8  | 22.5  |
| S.P. (Ring and Ball) of Residue, ° C.          | 35-70         | 49.0  | 39.2  | 51.7  | 62.5  | 60.6  |
| Penetration of Residue, 77° F., 100 g., 5 sec. |               | 43    |       |       | 17    | 20    |
| Penetration Index                              |               | -1.77 |       |       | -0.71 | -0.85 |

The air-blown residue used was the same as that used in Examples 1 and 2 above; the flux oil was the same as that described as starting material in the production of this air-blown residue; the distillate to 300° C. was prepared by distilling the above flux oil to a vapor temperature of 300° C., removing 22.3% of distillate by weight and using the distillate at the flux; the light carbolic oil used had the following properties:

Distillation to (° C.):

|         | Percent by weight |
|---------|-------------------|
| 210     | 0.0               |
| 235     | 0.6               |
| 270     | 75.0              |
| 315     | 89.0              |
| 355     | 94.1              |
| Residue | 5.0               |

The compositions of Examples 6 and 7 and of the standard RT-9 road tar were subjected to accelerated curing rate tests as follows:

An 8.00 gram portion of each tar was weighed into the lid of a 6-oz. Gill style ointment tin, this amount produced a film of 0.032 inch thickness corresponding to a road coverage of  $\frac{1}{3}$  gal./sq. yd. Nine such tins were prepared with each tar and one specimen from each series was carefully weighed. The specimens were placed in an oven, equipped with forced air circulation, and maintained at 50° C. At periodic intervals, one of each series of specimens was removed from the oven and the softening point determined. The carefully tarred specimens were weighed and returned to the oven.

30

Results:

TABLE V

| Elapsed Time Days | RT-9             |                  | Ex. 6            |                  | Ex. 7            |                  |
|-------------------|------------------|------------------|------------------|------------------|------------------|------------------|
|                   | Percent wt. Loss | S.P. (R&B), ° C. | Percent wt. Loss | S.P. (R&B), ° C. | Percent wt. Loss | S.P. (R&B), ° C. |
| 1                 | 3.0              | 24.7             | 2.6              | 27.6             | 3.3              | 25.9             |
| 2                 | 4.6              | 28.5             | 4.5              | 33.9             | 5.4              | 31.7             |
| 3                 | 5.9              |                  | 6.3              |                  | 7.2              |                  |
| 4                 | 6.7              | 33.7             | 7.5              | 42.4             | 8.3              | 43.3             |
| 7                 | 8.2              | 38.7             | 10.6             | 50.5             | 11.1             | 46.3             |
| 11                | 9.8              | 47.3             | 13.3             | 55.2             | 13.4             | 53.2             |
| 16                | 11.0             | 44.0             | 15.8             | 62.3             | 15.3             | 58.0             |
| 24                | 12.5             | 50.0             | 18.3             | 71.2             | 16.6             | 63.7             |

It will be noted from Table V that the road tars containing oxidized aromatic flux oil residue showed a much more rapid cure in that they attained ring and ball softening points of 40 and above in considerably shorter times than did the standard RT-6 road tar.

#### Examples 8 and 9

Two road tars were prepared by blending air-blown aromatic flux oil residue with a standard road tar in the proportions of approximately 70% and 45% by volume, respectively, of air-blown residue with 30% and 55% of the standard road tar and fluxing with a light carbolic oil residue to produce road tars containing 37.9 and 54.6 percent by volume of air-blown residue.

An 8044 gallon charge of aromatic flux oil having the following properties

Flux oil charge:

|                                                  |       |
|--------------------------------------------------|-------|
| Specific gravity at 100/60° F.                   | 1.099 |
| Water, percent by volume                         | 0.8   |
| D-246 distillation, percent by weight (to ° C.): |       |
| 235                                              | 0.0   |
| 270                                              | 9.6   |
| 315                                              | 37.9  |
| 355                                              | 70.5  |
| Residue                                          | 28.5  |

and with a light carbolic oil residue of the properties given below

#### Light carbolic oil residue (LCOR):

|                                                  |       |
|--------------------------------------------------|-------|
| Specific gravity at 100/60° F.                   | 1.029 |
| Water, percent by volume                         | 0.0   |
| D-246 distillation, percent by weight (to ° C.): |       |
| 170                                              | 0.0   |
| 235                                              | 2.1   |
| 270                                              | 79.4  |
| 300                                              | 89.8  |
| Residue                                          | 10.0  |

to form two blends as indicated below:

|    |                   |      |
|----|-------------------|------|
| 65 | Example No. 8     | Gal. |
|    | Air blown residue | 3699 |
|    | RT-9              | 1622 |
| 70 | LCOR              | 1456 |
| 75 | Example No. 9     | Gal. |
|    | Example No. 8     | 3777 |
|    | RT-9              | 1644 |

#### Example No. 9

The road tars thus prepared had the compositions and properties shown below:

## PHYSICAL CHARACTERISTICS OF ROAD TARS

|                                                      | RT-9  | Ex. 8 | Ex. 9 |
|------------------------------------------------------|-------|-------|-------|
| RT-9, percent by vol.                                | 100   | 23.9  | 47.2  |
| Air-blown Residue, percent by vol.                   |       | 54.6  | 37.9  |
| LCO R, percent by vol.                               |       | 21.5  | 14.9  |
| Float Test at 32° C., sec.                           | 154   | 185   | 161   |
| Soluble in CS <sub>2</sub> , percent TB, percent wt. | 89.8  | 88.6  | 85.0  |
| Specific Gravity at 25/25° C.                        | 1.212 | 1.190 | 1.198 |
| ASTM Distillation (D-20), percent by wt.:            |       |       |       |
| 0 to 170° C.                                         | 0.0   | 0.0   | 0.0   |
| 0 to 270° C.                                         | 8.0   | 13.0  | 10.7  |
| 0 to 300° C.                                         | 11.4  | 24.1  | 20.0  |
| Residue                                              |       |       |       |
| Ring and Ball Soft. Pt. of Res., ° C.                | 47.0  | 70.6  | 61.4  |

The standard RT-9 and the tars of the examples were tested for accelerated "cure" by the procedure described in Examples 4-7 above with the results shown below.

TABLE VI

| Time at 50° C., Days | Softening Point (R&B), ° C. |       |       |
|----------------------|-----------------------------|-------|-------|
|                      | RT-9                        | Ex. 8 | Ex. 9 |
| 1                    | 28.4                        | 30.2  | 27.5  |
| 2                    | 32.7                        | 36.5  | 35.2  |
| 4                    | 36.2                        | 44.0  | 40.4  |
| 7                    | 39.0                        | 50.5  | 46.6  |
| 11                   | 41.2                        | 57.2  | 52.0  |
| 15                   | 43.6                        | 61.0  | 54.9  |
| 18                   | 26.2                        | 63.2  | 57.5  |
| 21                   | 48.5                        | 68.0  | 58.4  |
| 24                   | 47.3                        | 64.3  | 60.4  |
| 37                   | 50.0                        | 71.7  | 60.6  |

It will be noted from Table VI that the road tars of the examples, containing oxidized aromatic flux oil residue are appreciably faster curing than the Standard RT-9 road tar in that they more rapidly attain high softening points than does the standard road tar.

The three tars described above were applied to different sections of the same road for test early in November. The road had been patched at the shoulders and was swept free of dirt and debris immediately prior to application of the tars. The weather was clear and the road surface dry. Example 8 was applied first to a portion of approximately 1,700 feet. This mix was applied at a temperature of 220° F. Example 9 was then applied, at a temperature of 210° F. from the first point over a second length of approximately 1,700 feet. Regular RT-9 was applied, at a temperature of 220° F., to a succeeding 1,700 ft. length.

All tars were applied at a coverage of  $\frac{1}{3}$  gallon per sq. yd. and  $\frac{3}{8}$ -inch cover stone was applied in the amount of approximately 30 lbs. per sq. yd. Any tar applied was immediately covered with stone and rolled to embed the stone firmly in the tar. The workmanship was excellent and the application all that could be desired. The initial behavior of all tars was identical.

Observation of the stretches of road to which the tars had been applied after elapse of ten months showed that the section treated with the normal road tar exhibited excessive bleeding and a surface from which a large proportion of the cover stone had been dislodged. Traffic areas had smooth oily surfaces.

The section treated with the tar of Example 8 which had the largest proportion of air-blown residue exhibited no signs of wear and no dislodgement of cover stone whatsoever and no signs of bleeding.

The section treated with the tar of Example 9 was in excellent condition with a major proportion of the stone still in place and showed only slight signs of bleeding.

It will be noted from the above examples that tars containing air-blown residue as defined will not only "cure" more rapidly than normal road tars, but will also have

residual films of higher softening points with good adhesion to cover stone and with little tendency to bleed and disengage from the stone aggregate.

## Example 10

To illustrate the superiority of the paving binders of the invention in producing "black bases" of higher stability under applied loads than normal road tars, two tars were prepared, one a Standard RT-6, the other a tar of the invention containing 45% of oxidized aromatic flux oil residue, having the constitution and properties set out below

|                                      | RT-6 (Control) | Example 10 |
|--------------------------------------|----------------|------------|
| Formulation:                         |                |            |
| Standard Road Tar                    | 100            | 42         |
| Carbolic Oil                         |                | 13         |
| Air-Blown Residue                    |                | 45         |
| Analysis:                            |                |            |
| Specific Viscosity (50° C./50° C.)   | 28.4           | 30.2       |
| H <sub>2</sub> O (Percent by volume) | 0.5            | 0.4        |
| Specific Gravity (60° F.)            | 1.200          | 1.189      |
| CS <sub>2</sub> Soluble, percent     | 10.00          | 12.37      |
| Distillation:                        |                |            |
| 0-200° C.                            | 0.0            | 0.0        |
| 0-235° C.                            | 4.5            | 0.5        |
| 0-270° C.                            | 13.4           | 14.7       |
| 0-300° C.                            | 20.8           | 26.7       |
| Residue ° C. (Ring and Ball)         | 38.0           | 43.0       |

Each of the tars described above, was mixed in proportions ranging from 96.5% to 94.5% with run-of-bank gravel having the following classification analysis using Standard U.S. Sieves:

|               | Percent |
|---------------|---------|
| 1½" sieve     | 100     |
| ¾" sieve      | 81.0    |
| No. 4 sieve   | 68.0    |
| No. 10 sieve  | 52.4    |
| No. 40 sieve  | 23.2    |
| No. 80 sieve  | 4.0     |
| No. 200 sieve | 1.5     |

The "black base" mixtures were prepared and tested according to AST test D-1559-58T for stability in the Marshall test machine. In this test, gravel and binder are mixed at elevated temperature and compacted in a mold to cylindrical test specimens. Test specimens are placed in the machine and subjected to a load applied laterally by means of a constant rate load jack until the maximum load is reached. This value is a measure of the maximum load the material will withstand before breaking takes place. Higher values indicate greater resistance to breaking, and thus indicate greater load bearing capacities. Results of tests on five mixtures containing different proportions of binder are shown in Table VII below.

TABLE VII.—MARSHALL STABILITY VALUES (ASTM D-1559-58T)

[Maximum load in pounds]

|    | Percent Binder | Percent Gravel | Standard RT-6 | Example 10 |
|----|----------------|----------------|---------------|------------|
| 60 | 5.5            | 94.5           | 696           | 958        |
|    | 5.0            | 95.0           | 673           | 827        |
|    | 4.5            | 95.5           | 859           | 987        |
|    | 4.0            | 96.0           | 840           | 1,244      |
| 65 | 3.5            | 96.5           | 762           | 1,134      |

It will be noted that the black bases made from RT-6 tar containing oxidized aromatic flux oil residue binder attain maximum stability with less binder than required for normal road tar, and that the maximum stability even at this reduced binder content is greater than the maximum that can be achieved with normal road tar. Stated another way, using the same amount of paving tar in both cases, the stability of the black base with the pre-oxidized binder is approximately 50% greater than that using the normal road tar.

While the above describes the preferred embodiments of the invention, it will be understood that departures may be made therefrom within the scope of the specification and claims.

I claim:

1. A paving tar composition consisting solely of coal tar derived products, said composition consisting essentially of a mixture of (1) between about 25% and about 75% by volume of a standard coal tar derived road tar as defined in A.S.T.M. standard specification D-490, and (2) between about 75% and about 25% by volume of a pitch-like oxidized aromatic coal tar flux oil residue obtained by contacting, with an oxygen-containing gas at temperatures between about 200° C. and about 500° C., a coal tar distillate boiling above about 250° C. selected from the group consisting of light and heavy coal tar oil fractions and residues from redistillation of lighter coal tar distillates and mixtures thereof, said contacting being continued for a time sufficient to provide a residue having a ring and ball softening point between about 40° C. and about 135° C. and containing between about 15% and about 45% of benzol insoluble compounds and not more than about 5% of quinoline insolubles, and having a penetration index between about 0 and about -1.5, said mixture being blended with (3) a minor amount of a coal tar distillate fluxing oil of which at least about 90% boils between about 210° C. and about 355° C., sufficient to bring the consistency of the resulting composition to within the viscosity requirements of road tar grade tar as specified in ASTM D-490.

2. The composition according to claim 1, wherein the fluxing oil is a light carbolic oil residue.

3. The composition according to claim 1, wherein the standard road tar-oxidized aromatic flux oil residue mixture contains between about 50% and about 75% by volume of oxidized flux oil residue, and wherein the fluxing oil is a light carbolic oil residue.

4. The composition according to claim 1, wherein the residue obtained by subjecting the said paving tar composition to distillation according to ASTM method D-20, has a penetration index of not less than about -1.0, and which residue is capable of setting to a ring and ball softening point of at least about 40° C. in not more than about 5 days when subjected, in a film of about .032 inch thickness to forced air circulation at 50° C.

5. The process for preparing a road tar composition consisting solely of coal tar derived products, said composition meeting the specifications of ASTM D-490 and having a low degree of temperature susceptibility and a rapid curing rate, which comprises blending (1) between about 25% and about 75% by volume of a standard coal tar derived road tar with (2) between about 75% and about 25% by volume of a pitch-like oxidized aromatic flux oil residue obtained by contacting with an oxygen-containing gas at temperatures between about 200° C. and about 500° C. a coal tar distillate boiling above about 250° C. selected from the group consisting of light and heavy coal tar oil fractions and residues from redistillation of lighter coal tar distillates and mixtures thereof, said residue containing between about 15% and about 30% by weight of benzol insoluble compounds and not more than about 5% of quinoline insoluble compounds, and having a ring and ball softening point between about 60° C. and about 75° C., and a penetration index not less than about -1.0 and fluxing the resulting blend with (3) a sufficient quantity of a coal tar distillate of which at least about 90% boils between about 210° C. and about 355° C. and having no more than about 10% residue above 355° C., to bring the consistency of the resulting composition within the viscosity requirements of at least one of the road tar grades as specified as ASTM D-490.

#### References Cited by the Examiner

#### UNITED STATES PATENTS

|              |         |                |        |            |
|--------------|---------|----------------|--------|------------|
| 2,395,041    | 2/1946  | Fair           | -----  | 196-14     |
| 2,521,783    | 9/1950  | Farber         | -----  | 106-283 XR |
| 2,701,217    | 2/1955  | Fair           | -----  | 117-113    |
| 35 2,772,219 | 11/1956 | Dunkel et al.  | 208-23 | XR         |
| 2,826,507    | 3/1958  | Waddill        | -----  | 106-284    |
| 2,888,357    | 5/1959  | Pittman et al. | -----  | 106-202    |
| 3,173,851    | 3/1965  | King et al.    | -----  | 208-23     |

40 ALEXANDER H. BRODMERKEL,

*Primary Examiner.*

MORRIS LEIBMAN, *Examiner.*

J. B. EVANS, *Assistant Examiner.*